

[72] Inventor Yoshio Mori  
Tokyo, Japan  
[21] Appl. No. 719,371  
[22] Filed April 8, 1968  
[45] Patented Dec. 8, 1970  
[73] Assignee Nippon Piston Ring Co., Ltd.  
Tokyo, Japan  
[32] Priority April 8, 1967  
[33] Japan  
[31] No. 42-28929

[56] References Cited  
UNITED STATES PATENTS

2,202,773 5/1940 Given ..... 123/90B1  
2,735,645 2/1956 Freed ..... 251/368X  
2,906,255 9/1959 Bonce ..... 123/188P  
2,973,183 2/1961 Alger ..... 308/N  
3,251,575 5/1966 Campbell ..... 251/368X

## FOREIGN PATENTS

868,925 10/1941 France ..... 123/90B1

Primary Examiner—Benjamin W. Wyche, III  
Attorney—Sughrue, Rothwell, Mion, Zinn & MacPeak

[54] VALVE LIFTER WITH THIN PLASTIC COATING  
2 Claims, 1 Drawing Fig.

[52] U.S. Cl. 123/90; 74/569  
[51] Int. Cl. F24c 3/00  
[50] Field of Search 74/569; 123/90(B); 251/368; 308/(N)

**ABSTRACT:** A valve lifter having mutually sliding surfaces requiring little or no lubrication, wherein at least one of said surfaces is coated with polytetrafluoroethylene.



PATENTED DEC 8 1970

3,545,415



INVENTOR  
Yoshio Mori

BY Siegmund Rothwell, Alan, Leon & Pfefferkorn

ATTORNEYS

## VALVE LIFTER WITH THIN PLASTIC COATING

## BACKGROUND OF THE INVENTION

This invention relates to construction of an improved valve lifter, particularly to a valve lifter for easy use in combustion engines.

Lubricating oil is normally supplied on the face where the valve lifter makes contact with the cam face and on the sliding surfaces where the valve lifter slides against a guide. It is usually necessary to wet the sliding parts of the valve lifter with a lubricating oil spread over the contact surfaces of metal at the start of the engine operation. Until the surfaces are adequately lubricated, scuffing, friction loss will occur. Engine performance is therefore substantially reduced at the start of its operation and considerable scuffing and abrasion by its sticking may result during these relatively brief periods. The problem has now become magnified with the advent of hard alloy-metal valve lifters for high speed rotation, since the harder the material is, the more abrasion and scuffing will occur at the beginning of the engine's operation.

## BRIEF DESCRIPTION OF THE DRAWING

The FIG. is a sectional side elevation of a valve lifter wherein the sliding surfaces are coated with polytetrafluoroethylene.

25

## SUMMARY OF THE INVENTION

It is an object of this invention to provide an improved valve lifter which is protected from scuffing and friction, and whereby the engine can be operated at peak efficiency from the start of its operation.

The objectives of this invention are achieved by coating the valve lifter with a film of polytetrafluoroethylene.

## DETAILED DESCRIPTION OF THE PREFERRED EMBODIMENTS

The drawing illustrating the invention is a sectional side elevation of the valve lifter and the cam, numeral 1 is the valve lifter, numeral 2 is the cam, numeral 3 is the cylinder block. The valve lifter, the cam and the sliding contact surface between the valve lifter and the mating guide portion are coated with polytetrafluoroethylene. The coating may be put on either the valve lifter and the cam or the contact surface of the valve lifter and the mating guide portion, since the polytetrafluoroethylene coated on one surface will partly adhere to the surfaces contacted therewith forming a film of the resin on the latter during the sliding contact. In the embodiment shown, the resin is coated onto the surface 4 and 5, whereby these surfaces contact with surfaces 4' and 5' respectively and a film of the resin is formed on the surfaces 4' and 5'.

The thickness of the film of polytetrafluoroethylene is not critical but it in general should be between about 5-300 $\mu$  ( $\mu$  = microns). The full effect however, will not be obtained if the thickness is under 5 $\mu$ . Over 300 $\mu$  the film often is loosened and might be removed by the sliding contact. Preferably, the thickness of the resin for the valve lifter of the combustion en-

gine for automobile, is about 10 $\mu$ .

The coating of polytetrafluoroethylene resin can be achieved by well known methods, i.e., flowing, spraying, enameling etc., but best results are obtainable by spraying.

5 Spraying is accomplished as follows: The valve lifter, cam, and mating guide portion are demated and their surfaces cleaned with water, liquid honed, and cleaned again with water to make it easier to adhere the resin. These are dried in the air. The aperture of the spray gun is suitably about 0.8-1.0 mm. 10 The coating liquid is made by using water, thinner or other solvents. The coating liquid should be agitated and passed through a filter of 100-200 mesh stainless wire. It is preferable to operate at the condition of 2-3 kg./cm.<sup>2</sup> spray pressure and at 15-20 cm. distance from the surface to be coated.

15 A suitable exhaust system is arranged in the place where the spraying is done and where it is kept clean without suspended matter such as dust.

After spraying, the member is dried in air or heated in air under 90° C. Infrared rays may be used for heating. Rapid drying

20 should be avoided to protect the film from forming wrinkles and cracking.

The member is then put into a furnace and baked at a temperature of 350-400 °C., and quenched whereby the film is made tenacious. The film of resin may be provided either on the surface 4 and 5 or on the surface 4' and 5', but it easier in operation to coat it on the surface 4 and 5 than 4' and 5'.

Polytetrafluoroethylene applied to the invention has a very small coefficient of friction, and also is so lubricous that it fully functions as a lubricant even if lubricating oil is not supplied.

30 Therefore, it does not happen that scuffing is caused at the contact surface of the valve lifter and the cam at the beginning of the running of the engine; also friction loss between the lifter and the guide is minimized.

In this way, a stable sliding between the surfaces is made possible providing a more fully effective engine even from the start of engine operation,

35 This invention can be adapted to the construction of any of various shapes and qualities of valve lifter i.e., it is applicable in the construction of valve lifter comprised as follows:

| 40 | Percent |      |      |       |       |      |      |      |      |
|----|---------|------|------|-------|-------|------|------|------|------|
|    | T.C     | Si   | Mn   | P     | S     | Ni   | Cr   | Mo   | B    |
| 45 | 2.80    | 1.80 | 0.50 | 0.30  | 0.10  | 0.20 | 0.30 | 0.20 | 0.02 |
|    | ~       | 2.80 | 1.00 | Below | Below | 0.80 | 1.00 | 0.80 | 0.10 |

50 I claim:

1. In an internal combustion engine having a rotating cam and a driven valve lifter having surfaces adapted for sliding contact with said rotating cam and with the block of said internal combustion engine, the improvement comprising a coating on at least one of said surfaces composed of a film of polytetrafluoroethylene having a thickness of from 5 to 300 $\mu$ .

55 2. The improved valve lifter as in claim 1, wherein the thickness of said film is about 10 microns.

60

65

70

75